

Jan. 28, 1936.

M. J. SHOEMAKER

2,029,131

WRAPPER OF TRANSPARENT OR ORNAMENTAL CHARACTER AND METHOD OF MAKING THE SAME

Filed May 27, 1931



## UNITED STATES PATENT OFFICE

2,029,131

## WRAPPER OF TRANSPARENT OR ORNAMENTAL CHARACTER AND METHOD OF MAKING THE SAME

Milton J. Shoemaker, Madison, Wis., assignor, by mesne assignments, to Carbide and Carbon Chemicals Corporation, New York, N. Y., a corporation of New York

Application May 27, 1931, Serial No. 540,375

16 Claims. (Cl. 93—2)

This invention relates to wrappers, of transparent or ornamental character, adapted to be applied to articles of commerce or containers therefor, and to the method of preparing and applying such wrappers. The wrappers may completely or partially enclose the article to be wrapped. A particular application of the invention is in the form of a new type of wrapper for covering or sealing closures for containers, especially bottles, jars, cans and the like. The closures may be in the forms of corks, rubber or other stoppers, screw tops, snap tops, pressed tops, and the like.

It is an object of the invention to provide a wrapper for containers and closures and other objects which may be applied in moist sheet or strip form and which shrinks upon drying to form a tight-fitting, smooth, glossy and attractive covering.

Another object of the invention is to provide a wrapper of this character in which the inherent adhesive properties of the wet sheet are sufficient to hold the overlapping portions together against the shrinking forces exerted.

It is a further object of the invention to provide a wrapper for containers and closures which cannot be removed without causing permanent, readily noticeable injury or defacement, thereby affording assurance to the user that the closure has not been tampered with and the container has not been opened.

It is a further object to provide wrappers for the closures of bottles, jars, cans and other containers of transparent or ornamental character in a manner such that pre-molding is not required.

It is a further object to provide a wrapper for container closures which is more simple to manufacture and to apply than present known performed bottle caps or wrappers of similar character.

An additional object is to provide a wrapper for containers or closures, which is considerably thinner than previously known wrappers for similar purposes, with the advantages that less material is required and also less time, heat, air circulation, etc., in the drying operation.

Other objects and advantages of the invention will become apparent as the following description progresses, which is to be considered in conjunction with the exemplary embodiments of the invention shown in the accompanying drawing wherein:

Fig. 1 is a front elevation of a bottle top showing the conditions which obtain immediately after

a strip of transparent film material is applied in moist condition to a bottle closure in accordance with my invention;

Fig. 2 is a similar view showing the conditions which obtain after the material has lost part of its contained water and has undergone partial shrinkage;

Fig. 3 is a similar view showing the wrapper after it has shrunk to its final proportions;

Fig. 4 is a top view of the portion of the bottle with the closure and wrapper which is shown in Fig. 3;

Fig. 5 is an end view, in perspective, of an article like an ordinary box which is being enclosed in a sheet of moist transparent film material, showing the folding of the edges thereof;

Fig. 6 is a similar view showing the edges after they are folded in place;

Fig. 7 is a front view of the same article after the transparent sheet has dried and shrunk upon it.

In the first four figures the dotted lines do not necessarily represent hidden lines but merely lines which are not upon the exposed surface.

Briefly, my invention comprises wrapping the article, or portion thereof or closure therefor which it is desired to seal or cover, with moist, distended film material in sheet form. In this connection the term "sheet" is used to include the different shapes the sheet may take, such as strips, ribbons, etc. The material preferably is arranged so that portions overlap and the overlapping portions are pressed together. It is then dried in air or in a suitable dryer and the shrinkage which accompanies the drying operation causes it to draw up very tightly against the adjacent surface of the enclosed object. Under proper conditions the material adheres to itself permanently at the overlapping portions to form a tight joint or seal without the use of special adhesive, and it also adheres to the adjacent surface of the object. The material used may be a cellulosic material having transparent film forming properties, such as many cellulose materials are known to possess. By cellulosic material is meant cellulose or a compound thereof. Other materials may be used, however, as will be more fully explained thereafter.

One of the preferred film forming materials is a hydroxyalphyl ether of cellulose, prepared as described in the pending application of A. W. Schorger, Serial No. 477,752, filed August 25, 1930, now Patent 1,863,208 issued June 14, 1932. Briefly, the ether is prepared by subjecting soda cellulose to the action of an olefine oxide. The

oxides at the lower end of the series especially those of ethylene and propylene produce the most practical cellulose derivatives. Of these the oxide of ethylene is preferred, because it is now more available commercially and is the cheaper of the two. The corresponding chlorhydrins may be used in place of the oxides. Glycerol monochlorhydrin may also be used.

When ethylene oxide or ethylene chlorhydrin is used it is preferable to keep the ethylene oxide content of the final product below about 20% of the cellulose used. Such ethers are cheaper because of their relatively high cellulose content, are tougher, stronger, and more flexible, are more resistant chemically, are easier to handle, are insoluble in water, have a more limited solubility in caustic soda solutions, that is, they are soluble in dilute solutions and substantially insoluble in concentrated solutions and are practically insoluble in caustic potash solutions. Ethers containing more than 20 per cent ethylene oxide are more or less water soluble, the solubility increasing as the oxide content increases. Controlled water solubility may be obtained by mixing definite proportions of the water insoluble and water soluble ethers.

The cellulose raw material, hereinafter called cellulose, is mercerized in a caustic alkali solution which is preferably substantially less than 50% caustic soda. After mercerization is complete, excess caustic soda solution is eliminated as by pressing, and ethylene oxide is brought into intimate contact with the wet alkali cellulose. The reaction is stopped when the desired amount of ethylene oxide, usually about from 7 to 20 per cent, has been absorbed by the alkali cellulose. I prefer to use about 12% ethylene oxide, based upon the weight of cellulose employed.

The product which probably is an impure hydroxy-alpha-ethyl ether of cellulose may be dissolved in a dilute caustic soda solution. My preferred concentration for a solvent is about 6½% caustic soda. The preferred ether concentration in the solution is from 6 to 7 per cent, but this may be varied if desirable. With ethers containing more than about 12% added oxide, solution is usually substantially complete but if small amounts of insoluble matter are present the solution may be filtered to render it clear. Because of the high viscosity of the solutions the filtering operation is tedious and often unsatisfactory and I prefer to subject the solution to a freezing operation described in A. W. Schorger Patent 1,941,277, issued December 26, 1933, based on application Serial No. 475,251 filed August 14, 1930, to render soluble the insoluble matter. With ethers made with less than about 12% added oxide this freezing operation is usually used because of the increasing amounts of insoluble cellulosic matter that may be present.

The unfrozen or the re-melted frozen solution may be extruded through suitable dies into a coagulating bath similar to that used in the viscose cellulose art. The material sets into a transparent non-fibrous flexible solid body. For the purposes of this invention the film or continuous sheet form of the material is used. The term "film" is used in the sense which excludes the filamentary form. After leaving the coagulating bath, the film may be run through one or more washing baths. The last washing bath may contain an agent for increasing the flexibility of the film, for instance, about 10 per cent glycerine. There may also be incorporated in the last bath a small proportion of a preservative, for instance, about 1% formaldehyde.

If it is desired that the film be opaque, a small proportion of a powdered pigment may be included in the solution of the cellulose ether in caustic soda. Pleasing effects may be obtained by incorporating small amounts, as low as a few per cent, of metallic powder, such as bronze powder, in the ether solution. If a colored film is desired any aniline dye which is suitable for dying viscose cellulose may be used.

In the foregoing and in the appended claims I have used the term "alpha-ethyl" as indicating a radical of the aliphatic series inasmuch as the term "alkyl" which is sometimes used to make this distinct reference is frequently indicative of both aliphatic and aromatic radicals. The term "alpha-ethyl" is specific to the aliphatic series in the same manner as "aryl" is specific to the aromatic series. See Richter's Organic Chemistry, Vol. 1, page 43, first English Edition 1916.

To utilize the film for the purpose set forth in this application the wet films which has been washed preferably is wound upon a reel or spool until a roll of sufficient size is obtained, a diameter of 6 to 10 inches being convenient. It is then enclosed in a water repellent wrapper or container, or placed in a moisture proof compartment. Here a small amount of water drains from the material. After this excess water has drained, the operation usually not requiring more than three or four days, the roll may be subdivided into rolls or discs of narrower widths if that is desirable. This may be done readily by means of any sharp-edged instrument, such as a knife, the material submitting to such cutting more readily when in this wet compact condition than when dry or when freshly formed. The reel upon which the material is rolled may be cut as well as the film so that the cut section of the reel may serve as a core to be mounted on a shaft for unwinding. The reels are usually of fibre board such as card board, which has been rendered water-resistant and which readily permits of cutting along with the film material.

The rolls may be of any desired width and the moist film material, in continuous sheet or ribbon form, is now ready for use in wrapping articles and container closures. If such operations are not to follow immediately, the rolls should be placed in moisture-proof inclosures which may be in the form of containers or compartments or moisture-proof paper wrappers and stored until needed. All of the water need not be retained but it is essential for satisfactory results that the material should contain at least 30 per cent water at the time it is applied as a wrapper. One of the distinct and novel advantages of my invention lies in the fact, mentioned above, that the wrapping material may be stored and shipped in moist condition within water-proof wrappers or containers or compartments as described above and can be preserved indefinitely in such condition. The material, preferably in roll form, may be stored, shipped and marketed as a useful article of commerce, to be applied by the user.

The formation of the material into closure wrappers for containers such as a bottle 9 in Fig. 1, will be described first. A length of the moist ribbon-like product somewhat greater than that required to encircle the top of the container closure is severed from a roll of the material. The severed strip is then rolled smoothly in lateral cylindrical encircling relation upon the container closure with the end portions overlapping. The top edge portion may extend above the closure and the bottom edge portion may extend

below the closure and encircle the adjacent portion of the container. The material is elastic and irregular contours are easily accommodated. The overlapping portions then are pressed together with normal pressure of the thumb or finger or the container may be grasped in the hand and the overlapping portions pressed against a resilient surface, such as a felt pad. The pressure need be only such a medium pressure as lends itself to convenient rapid operation. These operations may, of course, be done automatically.

Fig. 1 represents conditions which obtain immediately after the strip material 10, hereinafter called the wrapper for simplicity, has been applied to the closure 11 of the container 9. It encircles the closure 11 substantially in the form of a cylinder with ends overlapping an amount represented by the distance between lines 12 and 13. This may vary within wide limits but it is recommended that the overlap be not less than one-half inch. Of course, for a smaller size the overlap range may be less as the pull from shrinkage will be much less.

It may be desirable to encircle the closure several times. The top portion of wrapper 10 extends above the closure 11 and the bottom portion extends below it and encircles the adjacent portion of the neck 14 of the bottle. The bottle is now placed in a drying atmosphere where it dries and shrinks into final shape within an hour or two. If a current of warm air is directed upon the wrapper, less than 10 minutes is required for drying.

As drying continues the wrapper shrinks and Fig. 2 represents conditions which obtain after it has partially dried. It has lost some of its cylindrical shape and fits tightly against closure 11, the lower end portion having drawn in so that, instead of being spaced from the neck 14 of the bottle it is in contact therewith except for the tensioned spanning portion immediately below the flanged rim 15 of the closure. The upper end portion is drawn inwardly by shrinkage at an angle to the top of the closure. The shrinkage, however, ordinarily does not cause relative movement of the layers at the overlapping portion between lines 12 and 13.

Fig. 3 shows the wrapper after it has become air-dry and the shrinkage is substantially complete. The wrapper usually adheres to the closure and bottle neck and it follows closely the contour thereof. The upper projecting portion of the wrapper has become drawn down tightly against the top of the closure in the form of an annular ring 16 devoid of pleats as illustrated in Fig. 4. It is, of course, to be understood that the width of the ring 16 may be controlled to conform to the capacity for shrinkage to avoid forming pleats in the ring. The overlapping portions of the wrapper adhere to each other and do not permit of relative movement. The upper portion of the wrapper may be sufficiently large that when folded down upon the top of the closure the latter is completely covered.

It is to be understood that overlapping is not an essential requirement of the invention. Adhesive may be applied to the container closure or to the moist sheet material before the wrapping operation, in which case it is unnecessary to have portions of the material overlap. The same is true in connection with other articles which are to be wrapped or covered locally.

There are many other practical applications for wrappers of my moist sheet material. For

instance, where an article has a cover which is to be removed when the article is put into use, as is the case with certain types of dry batteries which have removable covers to protect the terminal leads, a strip of the wet film material may be wound around the article and cover so that the end portions overlap. Upon drying the strip holds the cover firmly in place.

It is also the purpose of my invention to enclose objects completely. Figs. 5, 6 and 7 illustrate the manner in which an object, in this case a frame containing honey in the comb, may be enclosed. A rectangular sheet of moist film material, such as has been described heretofore, is wrapped around the case 17 so that the two opposite end portions of the longer dimension overlap upon one side of the case, as is shown at 18, with the side portions of the sheet extending beyond the edges of the box or frame sides or ends. These are folded in an ordinary manner for wrapping packages. The narrow projecting portions of the sheet are then brought down flat against one side of the frame, as shown at 19 in Fig. 5. The necessary creases 20 are then pressed into the sheet and the wide projecting portions 21 are next folded flat against the side of the frame and the overlapping portions are pressed together. The same operations are repeated at the opposite side of the frame. The material usually is of the same thickness as when used for wrapping container closures.

Under proper conditions the inherent adhesive property of the moist sheet material is sufficient to keep the enclosure in substantially the form and position shown against the forces exerted by its shrinking action. Fig. 7 illustrates the appearance of the article. The honey comb 22 is clearly visible, the shrinking of the film during drying having drawn the latter smooth and taut, making it tight-fitting and imparting an attractive appearance to the article. As explained heretofore, adherent seals are formed at the seams or joints, and the product is protected against dust, insects, undesirable smells, loss of freshness and flavor, and to some extent against changes in atmospheric humidity conditions.

The illustration of a complete enclosure is merely one of a great many such applications for which my invention is suited. I have enclosed successfully articles such as bottles, containers of all kinds, toys, dolls, balls, such as golf and tennis and other kinds of rubber balls, articles of food, etc. I may use my improved wrappers and enclosures under any circumstances where a closely adherent, smooth transparent or decorative wrapper adds to the attractive qualities of articles of commerce and where cleanliness, sanitation, freshness and purity are desirable qualities. An attractive wrapping for angular or spherical objects has been made by winding a ribbon of the material about the object with the edge portion of each succeeding winding touching or overlapping slightly the edge portion of the preceding winding, this being continued until the object is completely covered.

As mentioned heretofore, I may use other film materials in addition to cellulose hydroxy-alkyl ether for my improved wrapper. Regenerated cellulose is suited to my purpose, particularly that regenerated from viscose, although I may also use cuprammonium cellulose and cellulose regenerated from cellulose nitrate and from cellulose acetate. Other film materials, such as cellulose acetate and cellulose nitrate, alkyl and other ethers of cellulose may be used but some are con-

sidered to be less desirable than those mentioned heretofore, because, when wet with water, they do not possess the same degree of the property of adhering to themselves or to the article covered. 5 This may be due to the fact that some are insoluble in water or aqueous solutions. It is necessary to apply an adhesive at the overlapping portions, or a small quantity of solvent for the film material may be applied. In one respect they are 10 all similar, in that they contain or may be wetted with a solvent or a liquid which penetrates the material to form an adhesive property.

The invention is not limited to cellulose and its derivatives. Other film-forming material may 15 be used. Gelatin films may also be used and wrappers of this material have been made.

The films usually are produced by shaping a viscous solution of the film-forming material into continuous sheet form and then coagulating or 20 hardening the material by passing it through a suitable coagulating bath. Gelatin solutions are hardened or tanned by means of solutions of formaldehyde or chromic salts. The film forming process must, of course, be adapted to the characteristics of the material. 25

The coagulated films are in the form of gels and contain large and rather definite quantities of water, depending upon the kind of material and method of manufacture. This water may 30 properly be designated water of gelation. The loss of this water is attended by pronounced shrinkage. When the dry films are soaked in water they absorb smaller quantities of water than they originally retained and lost on drying, 35 and they do not swell to their original dimensions. Upon subsequent drying, shrinkage is correspondingly less. It is therefore, important for the best results that such materials be initially undried.

For instance, cellulose hydroxy-alphyl ether 40 prepared as heretofore described, when freshly coagulated, contains about 88 per cent water. When the film is dried and allowed to shrink freely it shrinks as much as 35 per cent in length. When soaked in water the dry film absorbs at the 45 very most only about 75 per cent water. This actually is only about 40 per cent of the water which was contained in the freshly coagulated film. The swelling of the film is correspondingly less as is also the shrinkage which accompanies 50 subsequent drying. The other film materials act similarly but in varying degrees. With cellulose regenerated from viscose the proportion of water absorbed by the dry material is considerably less. A portion, therefore, of the water which was 55 originally contained in the freshly coagulated film does not re-enter the film after the latter has become dry and is subsequently soaked in water. This portion of the originally contained water may be called non-reentrant water of gelation.

All of the film materials herein named except cellulose hydroxy-alphyl ether are well known in the film making art and the methods for forming the moist films from solutions of the base materials are known and need not be described herein. The usual procedure in the manufacture of films from such materials includes a drying operation which follows immediately and continuously after the coagulating operation. In the preferred process of my invention the drying 60 operation is dispensed with and the newly-formed film, containing non-reentrant water of gelation, is rolled upon suitable spools, the spools cut into narrowed widths if desired and the resulting narrower rolls preserved in a sufficiently moist condition, preferably without substantial loss of

water, until it is desired to apply the film as a wrapper to an article. Methods for securing increased hardness or flexibility of films to best suit them for their functions are well known for each material. Methods of ornamentation are 5 also known and need not be described herein.

Of the film materials mentioned heretofore those which I prefer to use are cellulose hydroxy-alphyl ether and cellulose regenerated from viscose. The properties of films of these materials 10 are in general similar. When they contain the water from the forming operation they are distended, limp and tender and possess the property of adhering to themselves and to the surfaces of objects. Upon drying they shrink and gain 15 strength and stiffness. They do not possess these properties in equal degree but the differences are not sufficiently pronounced to require substantial variation in the conditions under which they may be applied successfully as wrappers. 20

The coagulated films usually contain 80 per cent or more of water. For instance, a cellulose hydroxy-alphyl ether film produced as described heretofore contains about 85 to 90 per cent water after the draining operation. A film of cellulose 25 coagulated from a solution of viscose containing about 5 per cent cellulose contains 85 per cent water or somewhat less. The water content is affected somewhat by the concentration of film-forming material in the solution from which the 30 film is coagulated and also by the incorporation of glycerine to increase flexibility. The optimum water content usually is considered to be that of the coagulated film which has not been allowed to dry to any appreciable extent because of the 35 superior adhesion and shrinkage obtained under such circumstances. Satisfactory results are obtained for most applications, however, with films containing as low as 75 per cent water. In the case of films which originally contained 85 to 90 40 per cent water this represents an actual decrease of from about 50 to 65 per cent of the original water.

With cellulose hydroxy-alphyl ether films it has been found that better adherence is obtained 45 if the film possesses slight water solubility. For this reason it may be desirable to mix a small quantity of water soluble ether with the water insoluble ether in the caustic soda solution.

For satisfactory results, the films for my im- 50 proved wrappers should not exceed a maximum thickness. The maximum thickness is determined by the difficulty encountered in securing satisfactory adherence at the overlapping portions with thick films without the use of excessive 55 and inconvenient pressure. Of course, adhesives may be used if desired but this is not the preferred method of application because of the inconvenience introduced by the added operation of applying the adhesive. When films are used which 60 are too thick there may be total failure of adherence with resulting separation at the joint, or the edges of the top overlapping portion may curl away from the bottom portion, producing an ob- 65 jectionable appearance. Another undesirable re- result is that the overlapping layers may be sepa- rated easily and the wrapper removed intact from the article and returned if desired with re- 70 sulting loss of the tamper proof qualities of the wrapper. This feature will be discussed more 70 fully hereinafter. With cellulose hydroxy alphyl ether films the maximum practical thickness is about .020 inch and with cellulose regenerated from viscose it is substantially the same or slight- 75 ly less because of the slightly increased stiffness

of this material. The foregoing figures are given for material which contains substantially all of the water of gelation from the forming operation. Maximum allowable thickness is less if the water content is appreciably reduced or if tamper proofness is a primary consideration.

It is advantageous to keep the film material thin because this permits conservation of material, reduction of time and expense of drying and results in improved adherence between layers. However, as the moist films become thinner they become weaker, more limp and tacky and are difficult to handle. The most suitable thickness, therefore, is that which combines economy with good handling properties and about .006 to .015 inch has been found to be a satisfactory thickness range for most materials. With cellulose hydroxy-alphyl ether and cellulose regenerated from viscose moist films of .008 inch thickness have been used with very good results.

When the proper thickness is used a good joint is secured at the overlapping portions by the use of normal pressure as heretofore described and the two layers adhere together sufficiently so that it is difficult to separate them without tearing the material of the layers. In the case of wrappers for container closures the material usually adheres sufficiently to the closure and the container so that it becomes torn in the removal operation. The wrapper, coming to the user in intact condition, is assurance to him that it has not been removed since it was applied and provides a convenient means for tamper-proofing containers and other articles.

The minimum thickness at which the moist films can be handled successfully is slightly less than the foregoing figures for the preferred thickness. For present day materials a thickness of about .005 inch is a practical minimum for successful wrappers. However, methods for making the moist materials tougher or stiffer may be developed in the future, in which case thinner films may be used.

With cellulose hydroxy-alphyl ether films it has been found that when applied as heretofore described, a moist film .008 inch thick shrinks to a thickness of about .001 inch at those points where shrinkage in area is substantially prevented. The drawings and description of the application of the wrappers to articles show that shrinkage in area usually is substantially prevented. For instance, in Fig. 1 the upper projecting portion of the closure wrapper is all that shrinks in area to any substantial amount. Where dry thickness is referred to in the description what is meant is the thickness at those points where the shrinkage in area is substantially prevented. The shrinkage of films of cellulose regenerated from viscose is less than that of cellulose hydroxy-alphyl ether films. Freshly prepared films, containing non-reentrant water of gelation, and being .008 inch thick resulted in a dry wrapper about .002 inch thick or slightly less. It has been found that the maximum dry thickness for satisfactory commercial production is about .0035 inch although wrappers can be made having a dry thickness of as much as about .005 inch.

In some cases dry films are suitable for starting material and will absorb enough moisture upon being soaked in water to produce the desired adhesion and shrinkage. This is the more satisfactory method for using gelatin films because of the greatly increased strength which is developed upon drying the tanned films. On

the other hand, those materials which are soluble in organic solvents such as cellulose acetate and some of the aryl and alkyl ethers of cellulose, absorb but little water after they have become dry and dry films are considered to be unsuitable for starting material. The conditions of application usually determine the suitability of moistened films. Where relatively less shrinkage is required they may be used. For instance, they may be used to wrap a frame of honey as shown in Figs. 5, 6 and 7 and also where it is desired to encircle an article with a band or tape or to hold a cover upon an article as described heretofore in connection with a dry battery. They may also be used for wrappers for container closures in many cases. For instance, the upper projecting portion of the wrapper as shown in Fig. 1 may be very small or may be omitted. In such cases reduced shrinkage is entirely sufficient to produce the desired close fitting relation between the wrapper and the closure and upper portion of the container. Where reduced shrinkage is sufficient freshly formed film material may be given a preliminary drying operation with results comparable to those obtained when dry films are moistened. It is considered that films containing less than 30 per cent water are unsuitable because they are deficient in the inherent adhesive power for use as a wrapper and require the application of adhesives.

In general, the properties of the moist films are affected by manufacturing conditions and other treatments. For instance, glycerine lowers shrinkage and impairs the adhesive power of the films. The figures given heretofore are for films which have been found to contain suitable proportions of glycerine, these proportions being from about 15 to 30 per cent in the dried film. The concentration of film-forming material in the solution from which the film is coagulated or hardened also affects the properties of the resulting film. The same is true with respect to the incorporation of materials for imparting opacity, color, ornamental effects, etc. While these effects influence somewhat the optimum thickness and other conditions of application of the films the information set forth heretofore gives a fairly accurate indication of those conditions under which satisfactory practical results are realized in most cases. However, the information is given to indicate the nature of the invention rather than to limit its scope.

While it is considered that cellulose regenerated from viscose and cellulose hydroxy-alphyl ethers are the most suitable and important film materials for my wrappers, the invention is broadly the application to articles or objects of moist film in the form of ribbons, bands, or sheets capable of shrinking into tight fitting relation with the article or object and capable of being caused to adhere readily to itself or to the article or object and any film material which may possess such properties is included within the scope of my invention.

My improved wrappers for container closures possess advantages over those which are known. The present practice with bottle caps made from cellulose regenerated from viscose is to mold them in thimble-like or ring-like forms. When freshly formed the material is about 0.030 inch in thickness and it shrinks upon drying to about .007 inch thickness. As pointed out, heretofore, the preferred thickness of my moist film material is not more than about .015 inch and the material shrinks to about .0035 inch or less in thickness.

upon drying. With cellulose hydroxy-alkyl ether, moist films about .008 inch in thickness are used commercially resulting in dry films about .001 inch thick. The result is a decided saving in material cost and in time and expense in connection with drying. The added thickness is required in the known types of bottle caps to provide body thereto to permit the necessary handling. Such caps are molded individually to the proper size and are shipped and stored in water until used. Such method of handling is less convenient than that employed in connection with my improved wrapper which is merely rolled up in moist condition, either with or without the non-reentrant water of gelation, and then unrolled by the user and cut into suitable lengths as needed. Due to the manner in which the water is held, the material is not unpleasantly wet to the touch but merely feels moist and is easy to handle.

I claim:

1. The process for forming a wrapper under tension upon an article which comprises wrapping upon at least a portion of said article a sheet of thin, limp, wet material having film-forming properties, said sheet being capable of shrinking substantially upon drying, arranging portions of said sheet in overlapping relation, pressing said overlapping portions together to cause adherence of the sheet portions, and drying said wrapper, the inherent adhesive properties of said wet sheet being sufficient to hold the overlapping portions together against the shrinking forces exerted by the shrinking action of the sheet.

2. The process for forming a wrapper under tension upon an article which comprises wrapping upon at least a portion of said article a thin, limp, wet sheet formed from material having film-forming properties, said sheet containing non-reentrant water of gelation and being capable of shrinking substantially upon drying, arranging portions of said sheet in overlapping relation, pressing said overlapping portions together to cause adherence of the sheet portions, and drying said sheet, the inherent adhesive properties of said wet sheet being sufficient to hold the overlapping portions together against the shrinking forces exerted by the shrinking action of the sheet.

3. The process for forming a tight-fitting wrapper upon an article which comprises wrapping upon at least a portion of said article a sheet of thin, limp, wet cellulose hydroxy-alkyl ether film containing non-reentrant water of gelation and being capable of shrinking substantially upon drying, arranging portions of said sheet in overlapping relation, pressing said overlapping portions together to cause adherence of the sheet portions, and drying said sheet, the inherent adhesive property of said wet sheet being sufficient to hold the overlapping portions together against the shrinking forces exerted by the shrinking action of the sheet.

4. The process for forming a tight-fitting wrapper upon an article which comprises wrapping upon at least a portion of said article a sheet of thin, limp, wet cellulose hydroxy-alkyl ether film which is capable of shrinking substantially upon drying, said sheet being not more than .020 inch in thickness, arranging portions of said film in overlapping relation, pressing said overlapping portions together to cause adherence of the sheet portions, and drying said wrapper, the inherent adhesive property of said wet sheet being sufficient to hold the overlapping portions together

against the shrinking forces exerted by the shrinking action of the sheet.

5. The process for forming in situ a closure wrapper for containers which comprises winding about the adjacent exterior portions of the closure and container a strip formed from material having film-forming properties which strip contains at least 30 per cent water and is capable of shrinking substantially upon drying, arranging portions of said strip in overlapping relation, pressing said overlapping portions together to cause adherence of the strip portions, and drying said wrapper, the inherent adhesive property of said wet sheet being sufficient to hold the overlapping portions together against the shrinking forces exerted by the shrinking action of the strip.

6. The process for forming in situ a closure wrapper for containers which comprises enveloping the adjacent exterior portions of the closure and container in a strip of cellulose hydroxy-alkyl ether sheet material, which strip contains non-reentrant water of gelation and is capable of shrinking substantially upon drying, arranging portions of said strip in overlapping relation, pressing said overlapping portions together to cause adherence of the strip portions, and drying said wrapper, the inherent adhesive property of said wet strip being sufficient to hold the overlapping portions together against the shrinking forces exerted by the shrinking action of the strip.

7. In the process of making a tight-fitting wrapper upon an article, the steps which comprise placing in overlapping relation sections of flexible sheet material not exceeding .020 inch in thickness and containing at least 30 per cent water, pressing said overlapping sections together to cause adherence of the sheet portions, and drying said sheet material the inherent adhesive property of said wet strip being sufficient to hold the overlapping portions together against the shrinking forces exerted by the shrinking action of the strip.

8. In the process of making a tight-fitting wrapper upon an article, the steps which comprise placing in overlapping relation portions of sheet cellulosic material not exceeding .020 inch in thickness and containing non-reentrant water of gelation, pressing said overlapping portions together to cause adherence of the sheet portions, and drying said sheet material, the inherent adhesive property of said wet strip being sufficient to hold the overlapping portions together against the shrinking forces exerted by the shrinking action of the strip.

9. The process of forming a tight-fitting wrapper upon an article which comprises wrapping a thin, limp, wet strip of material having film-forming properties upon said article, said material being capable of shrinking substantially upon drying, arranging portions of said strip in overlapping relation, pressing said overlapping portions together to cause adherence of the strip portions and drying said strip, the inherent adhesive property of said wet strip being sufficient to hold the overlapping portions together against the shrinking forces exerted by the shrinking action of the strip.

10. The process for forming in situ a tight-fitting closure wrapper upon a container having a closure provided with a skirt portion, which comprises winding in overlapping relationship about the skirt portion of said closure and the adjacent portion of said container a wet strip formed from material having film-forming properties, arrang-

ing a portion of said strip to extend above the top of said closure, said strip containing non-reentrant water of gelation and being capable of shrinking into tight contact with the skirt and top portions of said closure upon drying, pressing said overlapping portions together to cause adherence of the strip portions, and drying said strip, the inherent adhesive property of said wet strip being sufficient to hold the overlapping portions together against the shrinking forces exerted by the shrinking action of the strip.

11. A wrapped article comprising an article, a sheet of material having transparent film-forming properties wrapped upon said article and shrunk in tight-fitting contact therewith, said sheet being not more than .005 inch in thickness and having portions thereof in mutually overlapping relation, the inherent adhesive property of said sheet being sufficient to hold the overlapping portions together against the shrinking forces exerted by the shrinking action of the sheet.

12. A wrapped article comprising an article, a sheet or band of cellulose hydroxy-alphyl ether film material wrapped upon said article and shrunk into tight-fitting relation therewith, said sheet or band having portions thereof in mutually overlapping relation, the inherent adhesive property of said sheet being sufficient to hold the overlapping portions together against the shrinking forces exerted by the shrinking action of the sheet.

13. In combination, a container, a closure therefore, and a ribbon of material having film-forming properties wound upon adjacent portions of said container and said closure and shrunk in tight fitting relation to said container and closure, said ribbon having portions in mutually overlapping relation, the inherent adhesive properties of said ribbon being sufficient to hold the overlapping portions together against the shrinking forces exerted by the shrinking action of the material.

14. In combination, a container, a closure therefore, said closure having a skirt portion and a top portion at substantially right angles to said skirt portion, and a ribbon of material having film forming properties wound upon the skirt portion of said closure and the adjacent portion of said container, overlying the top portion of said closure and being shrunk in tight fitting relation to the surfaces of said container and closure, said ribbon having portions in mutually overlapping relation, the inherent adhesive properties of said ribbon being sufficient to hold the overlapping portions together against the shrinking forces exerted by the shrinking action of the material.

15. The process of forming a tight-fitting wrap- 15 per upon an article which comprises wrapping at least a portion of said article in a thin, limp, wet sheet of material having film-forming properties and a thickness varying between .005 to .015 of an inch, said sheet being capable of shrinking 20 substantially upon drying, arranging portions of said sheet in overlapping relation, pressing said overlapping portions together to cause adherence of the sheet portions, and drying said sheet, the inherent adhesive properties of said sheet being 25 sufficient to hold the overlapping portions together against the shrinking forces exerted by the shrinking action of the sheet.

16. The process of forming a tight-fitting wrap- 30 per upon an article which comprises wrapping at least a portion of said article in a thin, limp, wet sheet of material, portions of said sheet being arranged in overlapping relationship, said sheet of material being of such thickness that when it dries the adhesive properties of the ma- 35 terial are sufficient to hold the overlapping portions together against the shrinking forces exerted by the shrinkage action of the material, pressing said overlapping portions together to cause adherence of the sheet portions, and dry- 40 ing said sheet.

MILTON J. SHOEMAKER.